

## UNITED STATES PATENT OFFICE

2,015,690

## MANUFACTURE OF IRON ALLOYS

René Perrin, Paris, France, assignor to Société d'Electrochimie d'Electrometallurgie et des Acieries Electriques d'Ugine, Paris, France, a corporation of France

No Drawing. Application February 23, 1933,  
Serial No. 658,279. In France August 29, 1932

9 Claims. (Cl. 75—27)

This invention relates to improvements in the manufacture of iron alloys of very low carbon content.

The present application is a continuation-in-part of my application, Serial No. 584,584, filed January 2, 1932, which describes the treatment of metals with slags by violently intermixing the metal, while in a fluid molten state, with a fluid molten slag.

10 The production of iron alloys and in particular alloys with chromium and manganese, by the reducing action of carbon on the ore does not permit, even if the reducing agent is insufficient in quantity, of obtaining very low carbon contents. 15 During the first phase of the refining of the metal with respect to its carbon content by contact with the slag, which at that stage of the operation is highly oxidized because it is as yet insufficiently reduced, a considerable oxidation of the 20 useful element such as chromium or manganese for example takes place and a corresponding reduction in the quality of the alloy which, owing to this fact, ceases to comply with the required commercial standards.

25 Reduction by metallic reducing agents such as silicon, which may be alloyed with the basis element of the iron alloy of low carbon content to be produced, and in all cases devoid of carbon or nearly so, permits of the working up of these 30 low carbon alloys without introduction of carbon. It is necessary however, in the course of this operation, to eliminate almost the whole of the metallic reducing agent which tends to remain alloyed in part in the iron alloy to be produced. 35 This operation which is generally carried out by oxidation of the reducing agent at the expense of the oxygen of a slag charged with the oxides of the basis elements of the iron alloy which it is desired to produce, presents great difficulties.

40 The further the operation of eliminating the metallic reducing agent (the silicon for example) proceeds, the more the reducible oxides of the ore fused in the presence of the reducing agent are diluted by the oxides to which this metallic 45 reducing agent has given rise and by the bases intended to neutralize it so as to disturb the chemical equilibrium which tends to become established. The reaction becomes sluggish, and the exchanges between the bath of molten metal 50 and the slag take place more and more slowly. Slagging out becomes necessary in order to recharge a fresh quantity of ore rich in oxide and to fuse it in order to carry on the operation of elimination of the metallic reducing agent. These 55 slagging out operations followed by a fresh charge

clog the metallic bath which is the more refractory the nearer it comes to the refining desired.

Now it is known that the fusion of a metallic residuum in the electric furnace is difficult owing to the excessive conductivity of the metal. The consumption of kilowatts increases greatly owing to this fact and all the items of the net cost involved in such additional consumption of energy are proportionately increased. Moreover 10 the contact of the electrode or electrodes with the products to be fused is prolonged thus also producing a regular increase in the amount of carbon contained in proportion to the elimination of the metallic reducing agent by the reducible 15 oxides of the molten slag. Finally the prolonged heat at a very high temperature has a disastrous effect on the life of the linings and crowns of the furnaces.

To sum up: it may be observed that in the 20 course of the operation of eliminating the metallic reducing agent, the fusion is rapid at the beginning, facilitated as it is on the one hand by the high content of oxides in the ore to be fused (which disturbs the equilibrium in favour of a 25 rapid oxidation of the metallic reducing agent employed, accompanied by an evolution of heat brought about by the reaction) and on the other hand by the fusible oxidized compounds formed in the course of the reaction. The reaction then 30 becomes very sluggish and it becomes necessary to slag out in order to break up the equilibrium between the metal and the slag. The fusion of the second charge and of the succeeding charges if there are any, then proceeds very slowly because 35 the bath has lost much of its fluidity by the renewing of the slag and by the reduction of the amount of the reducing metal (silicon for example) to about 5% or less.

If it is desired to obtain alloys containing a very 40 small quantity of the reducing agent (0.50 or even 0.10%), several successive slaggings out will be necessary but they do not yield uniform results.

By means of the present invention these disadvantages may be avoided and in accordance 45 therewith are obtained rapidly and with regularity iron alloys (such as ferrochromium and ferromanganese for example) with a very low carbon content and with the elimination as completely as possible of the metallic reducing agent. 50

This invention consists substantially in bringing about in a continuous, rapid and intimate manner by the aid of violent intermixing, the contact of the molten metal with the oxidizing slag, the time taken to eliminate the reducing 55

agent being shorter the more intimate this contact.

In all cases, whether the slag passes through the metal or the metal is poured on to the slag, 5 the operation lasts only about a minute and there is no need at all to supply any external heat.

The oxidizing slag which is to act on the metal may be either previously melted in a suitable furnace, and be used in minimum quantity and 10 may be of a composition strictly determined in order that the equilibrium to be attained in the course of the violent intermixing shall correspond, in each case, to the practically total elimination of the metallic reducing agent associated 15 with the molten alloy to be worked, or it may be run from the furnace itself where the alloy has been produced, into a suitable ladle, and thereupon the metal remaining in the furnace may 20 be poured rapidly and in a thick jet upon the slag so as to produce a violent and turbulent intermixing of the slag and metal, as in the case of the "second example" described below.

It has been found in the case of iron alloys of 25 low carbon content obtained according to this invention that:

(1) The elimination of the metallic reducing agent during the very short period of time that the operation lasts, can be pushed as far as is 30 desired, that is to say until the residual content is comprised between 0.20 and 0.10 which permits of responding to all the requirements of steel manufacturers.

(2) By working always under similar conditions (composition and quantity of the metal and 35 of the slag in the presence thereof and also the mode of bringing them violently into intimate and rapid contact) the results are uniform and therefore avoid lower classifications of the castings.

These results are due to the fact that the new equilibrium (metal and slag) sought is practically attained throughout the entire mass simultaneously and this is proved by the fact that, if subsequently 45 the contact between the metal and the slag is prolonged, the amount of metallic reducing agent contained in the metal practically no longer changes.

The nature of the linings of the receptacle in 50 which this violent intermixing of the metal and the slag takes place has no influence on the desired reaction, the duration of the operation being too short.

The temperature of the metal is without any 55 great influence. It is sufficient that the metal be quite fluid at the commencement of the operation, the heat evolved in this latter permitting of retaining its fluidity unaffected up to the end.

If it be attempted to obtain ferro chromium 60 alloys for example by using silicon as the metallic reducing agent, it is possible by means of the present process either to obtain directly in a single operation and by the action of an oxidizing slag melted down separately, a ferrochromium alloy complying with current standards, that is 0.50 to 1% of Si, or to displace the state 65 of equilibrium in the direction of a removal of the silicon to a greater extent by violently intermixing the slag and the metal of a charge 70 composed of a mixture of silico-chromium, ore and bases, as soon as perfectly liquid fusion has been carried out, or finally to attain very extreme removal of the silicon (Fe-Cr<0.10Si) which a single operation does not permit of attaining. In 75 this latter case the metal which has been partly

desilicized (Si comprised between 0.50 and 1%) by the first violent intermixing operation is again violently intermixed with a slag which has been melted down separately and is highly oxidized. The slag which has thus acted on Fe-Cr with 1% of silicon as the maximum is used again for a first removal of silicon from a new heat of silico-chromium by violent intermixing. Said slag is in the meanwhile kept liquid in the furnace for the preparation of oxidizing slag for desilicizing. 10

The quantity of slag to be used will be merely a function of the amount of silicon contained in the ferro-silicon-chromium alloy from which the silicon is to be removed the amount of silicon contained therein being related to the amount of 15 carbon aimed at for the ferro-chromium alloy which is to be produced.

The violent intermixing of the mass of molten metal and oxidizing slag may be effected mechanically by a gas for example. This intermixing must be violent so as to limit the duration thereof.

It is possible also to carry it out in a simple and economical manner by using a casting ladle which first receives the slag, either melted down 25 separately, or run from the silico chromium alloy furnace or the like. The metal is then violently run in a thick jet on to the slag preferably from a considerable height and the slag finally comes to the surface which multiplies the surfaces of 30 contact between the metal and the slag. It is then found that despite the very short duration of the operation the elimination of the metallic reducing agent (silicon for example) is practically terminated as soon as the slag has collected 35 by decantation above the metal. The uniformity of the results obtained is perfect when attention is paid to the conditions of the respective weights of the metal and slag and the composition thereof. With ladles of the usual dimensions 40 the result is easily obtained.

Any means other than the ladle may also be used for carrying out the violent intermixing operation. The ladle is however the most advantageous because it affords the simplest means of 45 carrying out the operation in order to obtain a better result. There is every advantage in burning the silicon for example solely by reducing, if necessary, the associated oxides of the basis elements of the alloy rather than favouring 50 the elimination thereof by having recourse to the oxygen of the air.

I give below by way of examples which are not limitative some operations carried out in accordance with the present invention. 55

*First example.*—The removal of the silicon from 600 kg. of metal containing

|          |        |
|----------|--------|
| Silicon  | 48.35% |
| Iron     | 16.22% |
| Chromium | 35.20% |
| Carbon   | 0.082% |

was effected by means of 3200 kgs. of ore (forming an oxidizing slag) melted down in a furnace constructed for this purpose, and of the following 65 composition:

|                                |        |
|--------------------------------|--------|
| Cr <sub>2</sub> O <sub>3</sub> | 29.83% |
| Al <sub>2</sub> O <sub>3</sub> | 6.86%  |
| SiO <sub>2</sub>               | 3.21%  |
| CaO                            | 45.73% |
| FeO                            | 6.96%  |
| MgO                            | 7.25%  |

This oxidizing slag and the metal were run simultaneously and with violence into a ladle 75

which, as soon as it had received the constituents of the reaction, was taken to the foundry above the ingot moulds.

About four minutes elapsed between the commencement of the run into the ladle and the commencement of the casting of the metal into the ingot moulds.

The metal of the first ingot mould had the following composition:

|    |         |        |
|----|---------|--------|
| 10 | Silicon | 0.89%  |
|    | Carbon  | 0.068% |

980 kgs. of metal of a marketable composition were obtained in a single operation, and a very short one compared with that effected in a single furnace with the slag acting on the surface of the molten metal bath from which the silicon was to be removed.

*Second example.*—300 kg. of silico-chromium of the following composition

|          |        |
|----------|--------|
| Chromium | 37.20% |
| Iron     | 12.30% |
| Silicon  | 49.53% |
| Carbon   | 0.10%  |

were charged into a furnace together with 800 kg. of chromite mixed with 720 kg. of lime.

In this furnace a metal of the following composition was obtained:

|    |    |        |
|----|----|--------|
| 30 | Cr | 69.80% |
|    | Fe | 29.05% |
|    | Si | 0.51%  |
|    | C  | 0.08%  |

35 The slag was run into a ladle and when the slag had been run out of the furnace the metal remaining in the furnace was run rapidly and in a thick jet into the ladle. The metal mixed intimately with the slag with a vigorous and turbulent intermixing action.

The duration of the operation was one minute and the composition of the metal at the end of the operation was:

|    |    |        |
|----|----|--------|
| 45 | Cr | 70.50% |
|    | C  | 0.07%  |
|    | Si | 0.08%  |
|    | Fe | 28.90% |

50 In a few seconds therefore the removal of the silicon had been pushed very much further, owing to the intimate contact produced throughout between the metal from which the silicon was to be removed and the still oxidized slag, which was in contact in the furnace before evacuation into the ladle. This result could only have been obtained formerly with a complementary slagging out and a refining of about an hour without any certitude of obtaining the removal of the silicon to such a degree.

60 What I claim is:—

1. A process for manufacturing from an iron alloy containing a substantial amount of a reducing agent and having a very low carbon content, an alloy practically free of reducing agent, which consists in violently intermixing said alloy in a molten condition with a very fluid previously molten slag capable of oxidizing the reducing agent present in the alloy, the violence being such as to form an intimate mixture in a short period of time of the slag and the alloy, and separating the slag from the alloy freed of reducing agent.

2. A process for manufacturing from an iron alloy containing a substantial amount of silicon and very little carbon, an alloy practically free of silicon, which consists in violently intermixing

said alloy in a molten condition with a very fluid previously molten slag capable of oxidizing silicon, the violence being such as to intermix the slag intimately with the iron alloy, the operation being effected in such a short period of time as required to oxidize the reducing agent, and separating the slag from the desiliconized alloy.

3. A process for reducing to a very low extent the amount of reducing agent present in an iron alloy in a molten state, which consists in violently intermixing with the said iron alloy a very fluid previously molten oxidizing slag, the violence being such that in the short period of time required to oxidize the said reducing agent an intimate mixture of slag and alloy is effected, and separating the slag containing the oxidized reducing agent from the iron alloy.

4. A process for collecting in a slag in an oxidized condition a high percentage of a reducing agent present in an iron alloy, which consists in violently intermixing with said iron alloy in a molten condition a slag capable of oxidizing the said reducing agent and of dissolving the reducing agent oxide so formed, and separating the slag enriched in reducing agent oxide from the iron alloy.

5. A process for manufacturing an iron alloy practically freed of reducing agent and having a very low content of carbon which consists in imparting to a mass of a molten iron alloy containing a very low percentage of carbon and a high percentage of a reducing agent, a certain amount of kinetic energy and utilizing said energy for forcibly bringing together said iron alloy and a mass of very fluid molten oxidizing slag so as to atomize and violently intermix said slag with the iron alloy for such a period of time as to oxidize nearly instantaneously substantially the whole of the said reducing agent, and then separating the slag from the metal.

6. A process for manufacturing an iron alloy very poor in reducing agent and having a very low content of carbon, which consists in causing a mass of very fluid previously molten oxidizing slag to be violently intermixed in a state of fine division and for a short period of time with a mass of molten iron alloy containing a reducing agent in substantial proportion, and allowing the said finely divided slag to rise in and through the said iron alloy and to collect on the surface thereof.

7. A process for manufacturing an iron alloy very poor in reducing agent and having a very low content of carbon, which consists in treating in a furnace a raw iron alloy containing very little carbon and a high percentage of reducing agent by means of a very fluid oxidizing slag for such a period of time as to lower sensibly the content of reducing agent in the iron alloy and then violently intermixing the said slag and the said iron alloy for such a short period of time and with such a violence as to lower to a very small percentage the content of reducing agent of the iron alloy, and then separating the slag from the iron alloy.

8. A process for manufacturing an iron alloy having a very small content of reducing agent when starting from a mass of raw iron alloy having a high content of reducing agent, which consists in placing at the bottom of a ladle a mass of previously molten very fluid oxidizing slag and rapidly pouring the said mass of raw iron alloy in thick jet onto the said mass of slag with such violence as to cause a rapid intermixing to take place between the mass of alloy and the mass of slag within such a short period of time as required

to oxidize and to remove from the iron alloy into the slag the greater part of the reducing agent, and then separating the slag from the iron alloy.

5. 9. A process for manufacturing an iron alloy having a very low content of reducing agent by starting from a mass of raw iron alloy having a high content of reducing agent, which consists in

placing at the bottom of a ladle a mass of a previously molten very fluid oxidizing slag and pouring the said mass of raw iron alloy in thick jet and from a considerable height onto the said mass of slag, and then separating the slag from the iron alloy. 5

RENÉ PERRIN.